

March 1, 1932.

C. A. NICKLE

1,847,888

RESISTOR

Filed Aug. 9, 1929

Fig. 1.



Fig. 2.



Fig. 3.



Fig. 4.



Fig. 5.



Fig. 6.



Inventor:

Clifford A. Nickle,  
by Charles E. Tullar  
His Attorney.

## UNITED STATES PATENT OFFICE

CLIFFORD A. NICKLE, OF SCHENECTADY, NEW YORK, ASSIGNOR TO GENERAL ELECTRIC COMPANY, A CORPORATION OF NEW YORK

## RESISTOR

Application filed August 9, 1929. Serial No. 384,756.

5 My invention relates to electrical resistors and provides an improved resistor of the so-called self-reducing type, that is, one which has such a high negative temperature coefficient that its initial resistance is reduced to a relatively low value when its temperature is raised as by the heating effect of current passing therethrough. The invention also provides an improved method of making such 10 resistors as well as an improved terminal arrangement therefor.

15 Heretofore there has been a need for a satisfactory self-reducing resistor for use in motor starting circuits and the like where it is desired to provide a resistance of relatively 20 high value when the circuit is initially closed, which resistance is automatically reduced after the initiation of current flow in the circuit. Thus, in starting electric motors, the initial resistance of such a self-reducing resistor serves to limit the starting or inrush current of the motor at standstill and thereafter the heating effect of the current serves 25 automatically to decrease the resistance to a relatively low value after the motor is started. The simplicity of construction and operation of such an automatic self-reducing resistor current control arrangement obviously 30 renders it most desirable, if not ideal, for motor starting and other similar service.

35 Heretofore various materials have been proposed for use as self-reducing resistors, such, for example, as carbon, silicon, boron, copper oxide, magnetite, germanium, and various other substances and alloys.

40 However, as far as I am aware, all of the self-reducing resistors previously proposed have inherent deficiencies which render them more or less unsatisfactory for general commercial use. For example, many of the proposed self-reducing resistance materials are 45 inconsistent in the resistance values obtained therewith even when the conditions for manufacture are under control. That is, the resistor units even when produced as duplicates and in substantially the same manner have substantially different resistance values as well as different negative temperature coefficients of resistance. Also the self-reducing 50 resistance characteristics obtained with most

of the proposed materials is not nearly of the magnitude necessary to meet practical requirements. Furthermore, many of the proposed materials soon deteriorate in continued use so that while initially satisfactory 55 to some degree for the desired service, they gradually become unsatisfactory under continued service conditions. This is particularly true of the oxides and alloys which apparently change their resistance characteristics due to the repeated application of high 60 temperatures. Moreover, certain of the proposed materials may not even be operated at a high enough temperature to be effective without serious damage thereto. As a result, 65 it is impossible to produce a difference between the cold and hot resistance thereof of the magnitude required for practical use. Also many of the proposed materials are so 70 rare and expensive that general commercial use thereof in current controlling service is prohibitive from the standpoint of cost alone.

75 The principal object of the present invention is to overcome the difficulties heretofore encountered and provide a self-reducing resistance that will withstand relatively high temperatures; that will give a change of large magnitude between the cold and the hot resistance values; that will give consistent resistance values and characteristics 80 when manufactured and also after long continued service; and finally that may be manufactured cheaply enough to compete with other forms of current controlling devices now in commercial use.

85 Briefly, in accordance with the present invention, these results are obtained by forming the self-reducing resistor of tellurium.

In its ordinary commercial form, tellurium is a metal powder of about 99% purity. I 90 have found that this metal in solid form has a negative temperature coefficient of resistance such as to give a negative change in resistance of the order of 10:1 over a practical operating temperature range. Since the 95 metal melts at around 452 deg. C., a relatively high maximum temperature limit is permissible.

100 For certain service the self-reducing resistance elements may be formed by melting

the powdered tellurium and casting it into either a suitable container or into a self-sustaining form of resistance unit. However, I have found that in the self-sustaining cast form ordinarily the tellurium resistance units are too brittle and weak mechanically for general application. This is due probably to the fact that the melted tellurium as it cools after casting crystallizes into relatively large crystals, thereby producing a relatively fragile structure. However, I have found this difficulty may be overcome by hot pressing the powdered tellurium into a self-sustaining solid form at a temperature around or somewhat below the actual melting temperature. The hot pressed tellurium has a micro-crystalline structure of substantially uniform resistance characteristic when manufactured under uniform temperature and pressure conditions. Furthermore, the micro-crystalline structure of the hot pressed body of tellurium provides such substantial mechanical strength that it not only is self-supporting and hence needs no container, but it is not easily broken by jars or shocks and will withstand even quite rough usage, such, for example, as dropping it on the floor. Moreover, the micro-crystalline tellurium possesses such a relatively high initial resistance value that solid units of large cross-sectional area may be employed, thus providing not only increased mechanical strength but also sufficient heat storage capacity to control the increase in temperature and thereby delay the automatic decrease in the self-reducing resistance for a desired time interval after the flow of current therethrough is initiated.

The invention is illustrated in the accompanying drawings, in which Fig. 1 is a perspective view of a tellurium self-reducing resistance unit having an improved form of terminal connector, Fig. 2 shows schematically one way in which the powdered tellurium may be hot pressed into the self-reducing resistance units, such as shown in Fig. 1, Fig. 3 is a circuit diagram showing a plurality of the tellurium self-reducing resistor units connected in series in the starting circuit of a split phase type of alternating current induction motor, Figs. 4 and 5 are circuit diagrams showing the tellurium self-reducing resistors applied for starting three-phase alternating current induction motors, and Fig. 6 shows the resistors connected in a tungsten lamp circuit for controlling the inrush current.

The self-reducing resistor unit 10 shown in Fig. 1 is formed of tellurium hot pressed into a solid rod in the manner described in connection with Fig. 2.

The tellurium resistance unit 10 is provided with the screw-threaded terminals 11 and 12, preferably formed of iron and having suitable nuts 13 thereon for securing the circuit conductors to the resistance unit and establishing good electrical contact therewith.

While the terminal construction just described is preferable, terminals also may be provided by electroplating the ends of the resistor unit or by hot pressing other good conducting material, such as iron powder, into the ends of the resistor unit. For the larger size units, the terminals may be clamped under pressure around the ends of the tellurium rod.

Since the resistance of the tellurium is relatively high, being of the order of 2,000,000 ohms per mil foot at normal room temperature, the cross section of the resistance unit may be relatively large. This permits a unit of substantial size and mechanical strength to be employed, even where comparatively high resistance values are desired.

The cross sectional shape of the resistor 10 depends upon the particular form of the mold in which it is hot pressed, and may be round, square, or any other desired shape. However, the resistor 10 preferably is of circular cross section when made in the manner illustrated in Fig. 2.

In this figure the mold 14 may be formed of fused quartz so as to withstand high temperatures, and is provided with a slightly tapering cylindrical bore 15 for receiving the powdered tellurium to be hot pressed. The fused quartz mold is better than a mold formed of metal, for the reason that it does not tend to alloy or adhere to the powdered tellurium during the hot pressing process.

The mold 14 rests upon a base 16 which also may be formed of fused quartz with the tapering bore 15 increasing in diameter from the top to the bottom. The iron terminal screw 12 is placed in a suitable recess formed in the base 16 and extends partially into the bore 15 so as to be embedded in the end of the tellurium unit as it is hot pressed. The screw terminal 11 is located in a similar manner in the plunger 17 by means of which pressure is applied to the powdered tellurium during the hot pressing process.

The bore 15 is then filled with powdered tellurium with the mold heated by any suitable means, not shown, to a temperature around or somewhat below the melting temperature of the tellurium. I have found that the precise temperature employed is not critical but may be anywhere within the range from just below the melting point to the temperature at which the tellurium powder just begins to soften.

Pressure then is applied to the plunger 17 with the heated tellurium in a plastic state. As a result, the volume of the powdered tellurium is reduced by about one-half, as indicated by the dotted lines in Fig. 2. During the compression of the plastic tellurium the terminal screws 11 and 12 are firmly embedded into the ends of the resistor unit. Furthermore, I have found that the embedded ends of the iron terminals are thor-

oughly wetted by the plastic tellurium, thus establishing a good current conducting relationship therebetween. I have found that the iron terminal screws are the most satisfactory, although other forms of terminals may be employed if desired.

The base 16 is then removed and the hot pressed tellurium resistor unit is readily forced out of the bottom of the tapered bore

15 in the solid mold 14. Due to the tapering shape of the bore 15, the tendency of the plastic tellurium to adhere to the walls of the mold during the compressive operation is materially decreased. This insures a practically uniform pressure application throughout the entire length of the resistor unit. The taper also readily permits the removal of the completed unit as just described. It will be evident, however, that other forms of molds may be employed, as, for example, any of the ordinary forms of split molds.

The tellurium resistor unit formed in the above manner is mechanically strong even when removed hot from the mold, and has a 25 very fine micro-crystalline grain structure.

While I have obtained the best results by hot pressing the powdered tellurium in the manner just described, the tellurium resistor units also may be made by casting the melted tellurium in a hollow container of suitable shape or by cold pressing the powdered metal under heavy pressure and then sintering the compressed billets. I have found, however, that the hot pressing imparts greater mechanical strength due to the micro-crystalline structure obtained and in addition insures resistor units of precisely the desired shape with a nicely finished surface. Also, the application of the resistor terminals is facilitated by the hot pressing method.

Fig. 3 shows the self-reducing tellurium resistor units employed in the starting circuit of a split phase type of alternating current induction motor, such as used in domestic electric refrigerators. The motor has a running winding 20 and a starting winding 21, both acting upon the squirrel cage rotor 22. The energizing circuit of the motor is controlled by the switch mechanism 23 which may be of the form described and claimed in the Hutt Patent 1,637,042 having a temperature responsive operating element 24 and an overload protective element 25 and a manual operating element 26. The self-reducing tellurium resistor 10 is connected in series circuit with the starting winding 21, which circuit is controlled by the normally open relay 27 having an operating winding 28 connected in circuit with the running winding 20.

With this arrangement, upon closure of the control switch mechanism 23, to start the motor, the inrush current through the running winding 20 closes the starting relay 27, thereby energizing the starting winding 21 through the self-reducing tellurium resistors

10. The particular function of the self-reducing tellurium resistor in this service is to compensate for variations in the line voltage. Thus, with normal or high voltage, the self-reducing tellurium resistors serve to limit the current supplied to the starting winding to a permissible value such as to avoid flickering in the lighting circuit on which the electric refrigerator may be used.

In case of low voltage such that the motor does not readily start with the limited current through the starting winding, the self-reducing tellurium resistors automatically decrease their resistance due to the heating effect of the current flow therethrough until sufficient current is obtained to insure starting of the motor. This automatic reduction of the resistors 10 occurs before the thermal overload element 25 has time to function. Thus, with the self-reducing tellurium resistors of the present invention the starting of the refrigerator motor is assured under all voltage conditions, and at the same time excessive starting currents on normal or high voltage such as to flicker the lights are effectively avoided.

In Fig. 4, the self-reducing tellurium resistors 10 are connected in each line of the three phase induction motor 30 and serve to reduce the voltage applied to the motor 30 in starting to a desired value. As the motor starts and reaches running speed, the heating effect of the current flowing through the resistors 10 causes the initial resistance thereof practically to disappear and thereby impress substantially full line voltage on the motor 30.

In Fig. 5, the self-reducing tellurium resistors 10 are connected in the secondary or rotor circuit of a three-phase wound rotor type of induction motor 31. Thus, in starting the resistors 10 are of relatively high value to provide a good starting torque, and as the motor starts and comes up to speed the resistance is decreased to provide efficient operation with normal running torque.

In Fig. 6, the self-reducing tellurium resistor 10 is connected in circuit with a plurality of tungsten lamps 32 in order to compensate for the marked positive temperature coefficient of these devices. Upon closing the lamp circuit the resistor 10 limits the inrush current and the resulting heating effect of the current reduces the resistor 10 and at the same time increases the resistance of the lamps to the full value.

It will be apparent to those skilled in the art that my improved form of self-reducing resistor may be employed with advantage in many other fields of service.

What I claim as new and desire to secure by Letters Patent of the United States, is:

1. A self-reducing resistance for electric circuits composed of micro-crystalline tellurium.

2. A self-reducing resistor for electric cir-

cuits comprising tellurium formed into a micro-crystalline solid body.

3. A self-reducing resistance for electric circuits consisting of a self-sustaining body of micro-crystalline tellurium.

4. A resistor unit composed of a mass of tellurium formed by pressure and heat into a micro-crystalline solid body.

5. A resistor unit consisting of a self-sustaining rod of micro-crystalline tellurium with metallic terminals embedded in the ends thereof.

6. The method of forming tellurium resistor units consisting of heating a powdered mass of tellurium to a temperature below the melting point and applying pressure to solidify the mass.

7. The method of forming resistor units consisting of embedding solid metallic terminals in a mass of powdered tellurium, heating the mass to a temperature at which the tellurium wets the terminals, and applying pressure to solidify the mass about the terminals.

In witness whereof, I have hereunto set my hand this 8th day of August, 1929.

CLIFFORD A. NICKLE.